

## UNITED STATES PATENT OFFICE

1,922,709

## PROCESS FOR MANUFACTURING NITRO-COMPOUNDS

James F. O'Brien, Seattle, Wash.

No Drawing. Application December 20, 1927  
Serial No. 241,463

2 Claims. (Cl. 260—142)

This invention relates to a process for manufacturing nitro-compounds from coal tar oils and relates more particularly to a process for nitrating and refining the light oil obtained from 5 coal tar distillation, at temperatures from 95° to 115° Centigrade, whereby such oil may be utilized as a hydro-carbon for explosives employing oxidizing bases, such as salts of alkaline metals, ammonium, or the like.

10 The primary aim and fundamental object of the present invention is the provision of a low temperature nitration process for treating light oil of coal tar, whereby a greater yield of low freezing and water-proofing properties and qualities for the refined nitrated product is obtained.

The present process contemplates increasing the specific gravity of the light oil by the reflux distillation process; removing the fatty matter contained therein nitrating the refined oil liquor at low temperatures combined with rapid increases of temperatures after nitration and the retention of such increased temperatures for predetermined periods; neutralizing the nitrated oil; and finally washing the same, all of 25 which are important features and objects of the invention and are to be correlated in the broad aim of enhancing the efficiency of the process for general use, and for producing a hydro-carbon for explosives which will remain 30 liquid at all ordinary temperatures.

The above, and additional features, purposes and advantages, which will hereinafter be more specifically treated, are attained in the manner set forth in the following specification and then 35 more clearly pointed out in the claims, which are appended hereto and form part of this application.

Before taking up the detailed description of the process and product evolved by the present 40 invention, a general exposition of the advantages and benefits to be derived therefrom will be undertaken.

Heretofore mononitrotoluol, dinitrotoluol and trinitrotoluol have been generally employed as 45 hydro-carbons for chlorate explosives, and in their commercial form ordinarily contain certain substances having no essential value, insofar as the efficiency of the explosives is concerned, and for this reason have, in some instances, been used to the extent of 90% filler. Further, the toluols above named contain such a large percentage of impurities as to materially decrease their efficiency, and in addition thereto materially affect their water-proofing and low freezing 50 properties and qualities. It is therefore, a

primary object of this invention, to provide a process for treating the light oil obtained from coal tar at temperatures between 95° to 115° Centigrade and having an average specific gravity of approximately .862, whereby a novel liquid 60 hydro-carbon is produced, which is neither a mononitrotoluol, dinitrotoluol, or trinitrotoluol, but which possesses greater waterproofing properties and the same non-freezing properties as dinitrotoluol, and which may be employed as an 65 insulator and desensitizing agent for any salts of alkaline metals, ammonium, or the like used as explosive oxidizing bases.

In carrying out the process in its preferred embodiment, the light oil distilled from coal tar at 70 temperatures from 95° to 115° Centigrade and having an average specific gravity of approximately .862, is first treated by the reflux distillation process to raise its specific gravity to .904, and for this purpose a vacuum still having 75 a reflux condenser, a steam coil and cooling coil is employed and charged with the light oil to be treated. A loss of approximately 20% of light oil volume occurs during distillation, so that a specific gravity of .904 is obtained for the resultant oil liquor; which is then subjected to the action of  $\frac{1}{2}$  to 1% strong sulphuric acid solution to 80 destroy the foreign fatty matter contained therein; then cooled off to approximately 20° Centigrade, then prenitrated with a solution of nitric 85 acid, sulphuric acid and water in the following proportions: 70%  $H_2SO_4$ , 20%  $HNO_3$  and 10%  $H_2O$ , the amount employed being 5% by volume of oil liquor. The acid solution is added very slowly and the temperature of the oil liquor during this time must not exceed 20° Centigrade, 90 and when the desired amount of acid solution has been added, the temperature of the oil liquor and acid mixture is increased to 70° Centigrade for one-half hour, following which it is decreased 95 to 30° Centigrade.

The oil liquor is then allowed to settle and the spent acid is run off, then the oil liquor is treated with a 2% solution of caustic soda, then it is washed with water in the following proportions, 100 10 parts of water to 1 part of oil liquor, following which it is allowed to completely settle for approximately eight hours, at which time pre-nitration of the same is completed.

The prenitrated oil liquor is next blown to a 105 gravity feed tank above a nitrating vessel, which latter is charged with an acid solution consisting of 60%  $H_2SO_4$ , 35%  $HNO_3$  and 5%  $H_2O$ . The prenitrated oil liquor is slowly added to the acid solution, in the proportion of  $\frac{1}{2}$  oil liquor to  $\frac{1}{3}$  110

acid solution, the temperature being maintained at 20° Centigrade and when all of the oil liquor has been added the temperature is increased by means of a steam coil in the nitrating vessel to 5 70° Centigrade for approximately one-half hour, the intermixed charge being kept in motion during this time, following which the same is cooled to 20° Centigrade, and is then allowed to settle for approximately four hours. The dinitrated 10 oil liquor is then drawn off into a neutralizing tank and is washed with a 2% to 5% neutralizing solution, such as caustic soda, soda carbonate, or lime, until a neutral point is reached, following which the neutralized-dinitrated oil liquor 15 is washed with hot water at 65° Centigrade for approximately one-half hour, after which it is allowed to settle for approximately two hours, this completes the nitration process. In this connection I desire to state, that the spent acids upon 20 completion of the dinitrating of the oil liquor are run off to a rectifying tank and are used again for the prenitration of succeeding charges of oil liquor.

The resultant dinitrated product, which I have 25 elected to name "Toluite" is neither a mono-nitrotoluol, dinitrotoluol, or trinitrotoluol, consisting as it does of approximately 39% ortho-nitrotoluol, approximately 58% para-nitrotoluol and approximately 3% miscellaneous hydrocarbon 30 matter, having an average specific gravity of 1.44 at 30° centigrade, and has a formula  $C_7H_6N_2O_3$  as compared with dinitrotoluol having a formula  $C_7H_6N_2O_4$ , and a specific gravity of 1.02 in its commercial form.

35 The "Toluite" of the invention contains all of the waterproofing and low freezing properties and qualities of ortho-nitrotoluol and para-nitrotoluol and at the same time the benzol and benzene elements are not in ratio to be harmful to 40 the strength of the explosives with which the "Toluite" is used, nor does actual experience show that the flame of such explosives is increased.

The essentials and important features of the 45 present process and product are the specific gravities of the light oil (.862), the  $H_2SO_4$  (1.84), and the  $HNO_3$  (1.44); employment of reflux distillation, and the employment of lower temperatures of nitration, as compared with the distillation methods and higher temperatures of nitration 50 heretofore employed in other nitration processes. Actual experience has demonstrated that the lower the point of nitration the greater the yield of low freezing and water-proofing properties and qualities of the resultant product, and by 55 rapidly increasing the temperatures and holding same for predetermined periods after nitration, in accordance with the time-temperature steps herein set forth, the larger final yield of refined dinitrated oil liquor is obtained. The yield of 60 refined dinitrated oil liquor to the raw oil should be substantially in the ratio of one and one-half gallons of refined oil to one gallon of raw or light oil, due primarily to the absorption or the incorporation of acids therewith while being treated.

65 In the production or manufacture of explosives the novel dinitrated oil product or hydrocarbon "Toluite" functions as the sensitizing agent therefor, and for this purpose is intimately intermixed with oxidizing agents, such as chlorates or perchlorates of alkaline metals, or of ammonium, together with carbonaceous substances, and with or without nitrates of the alkaline metals, or of ammonium, and with or without restrainers, such as silico-aluminous substances and 70 carbonates of the alkaline earths, and with or

without further water-proofing agents, such as collodion or collodion cotton, and with or without agents, such as dehydrated sodium carbonate in powdered form, whereby the deliquescent salts, occurring as impurities in the said chlorates and perchlorates, are converted into non-deliquescent salts, which will not subsequently absorb water and thereby materially affect or injure the quality of the explosives. While the primary function of the "Toluite" in the explosives is to sensitize the oxidizing agents or substances in their general explosive reaction, as above described, it also serves due to its oily nature to desensitize said agents against mechanical friction during processing of the explosive by coating or insulating the crystals of the same, whereby the resultant explosive compounds possess the following inherent qualities and attributes: they cannot be detonated by shock, vibration or jar, friction, nor by percussion unless a high degree of heat is developed; are non-deteriorating and non-deliquescent; if ignited without percussion in the open, or unconfined, burn extremely slowly as pieces of harmless fuel; require fulminate of mercury caps of high power, as for example 6 x caps, 100 for detonation either confined or unconfined; are substantially smokeless, except for minimum amounts of non-injurious fumes; are easily, safely and economically manufactured and prepared for commercial use in the form of plastic cartridges or sticks of suitable consistency in various degrees of strength and speed of detonation from the range of black powder to that of high explosives, and are adaptable for hard rock mining, 105 stump blasting, road work, quarrying, tree planting, ditching, breaking up hard-pan, "bulldozing", as a low flame powder for coal mining, and being substantially free from noxious gases or fumes, as above mentioned, are especially adaptable and desirable for use and employment 110 in constricted and confined spaces.

To further increase the speed of detonation of the explosives herein described I may elect to combine therewith an additional hydro-carbon or nitro-compound, such as trinitrotoluene, nitroglycerine or the like, which compounds are intimately intermixed with the "Toluite" prior to its incorporation with the correlated oxidizing agent thereof.

In the practical manufacture of the explosives 125 for various uses and purposes, I have found the following formulae to be very effective for rock blasting and stump blasting explosives.

| Rock blasting explosive No. 1 |          |
|-------------------------------|----------|
|                               | Per cent |
| Sodium chlorate               | 78       |
| Toluite                       | 15       |
| Sawdust                       | 7 135    |

| Rock blasting explosive No. 2 |          |
|-------------------------------|----------|
|                               | Per cent |
| Sodium chlorate               | 73 140   |
| Sodium nitrate                | 7        |
| Toluite                       | 15       |
| Sawdust                       | 5        |

| Stump blasting explosive No. 1 |          |
|--------------------------------|----------|
|                                | Per cent |
| Sodium chlorate                | 40       |
| Sodium nitrate                 | 38       |
| Toluite                        | 15 150   |
| Sawdust                        | 7        |

## Stump blasting explosive No. 2

|                 | Per cent |
|-----------------|----------|
| Sodium chlorate | 33       |
| Sodium nitrate  | 40       |
| 5 Toluite       | 18       |
| Sawdust         | 9        |

Wherefore, it will be manifest and apparent to those skilled in the art upon an understanding of the foregoing, that the present application is predicated upon the disclosure of a process for manufacturing nitro-compounds from light oils distilled from coal tar at temperatures ranging between 95° to 115° Centigrade and having an average specific gravity of approximately .862: which contemplates employing reflux distillation of such oils; nitration of the same at low temperatures combined with rapid increases of temperatures after nitration and the retention of such increased temperatures for predetermined periods, thus evolving a novel time-temperature nitration method for the production of a novel nitro-compound therefrom having a greater percentage of waterproofing and non-freezing properties and qualities than heretofore obtained, and which will remain liquid at all ordinary temperatures. The invention further contemplates the disclosure of explosive compounds embodying the novel nitro-compound hereinbefore described, which latter, due to its specific characteristics, interacts when combined or intimately admixed with certain specific oxidizing salts and other suitable ingredients to produce essentially new explosive compounds possessing certain novel characteristics in both their static form and their explosion. However, it is to be understood that the invention resides in the novel compositions of matter having these distinctive attributes, and that they therefore are not limited to the particular ingredients herein mentioned, or their specific proportions, as I am aware that substitutions may be made in the constituent ingredients, and variations in their proportions without essential modification of the resulting compositions. The relative proportions of the several ingredients may be varied within reasonable limits according to the special application for which the explosive is desired, as in some instances a high explosive is necessary, while, in other instances a rather retarded or slower effect is desirable, the former effect is obtained by increasing the percentage of chlorate in the composition, while the latter effect is secured by decreasing the percentage of the same.

Having thus fully described my invention, what I claim as new and desire to secure by Letters Patent is:

1. The process of manufacturing a nitro-compound which comprises distilling coal tar at temperatures ranging approximately from 95° to 115° centigrade to produce a light oil therefrom having an average specific gravity of approximately .862, raising the specific gravity of such light

oil by reflux distillation to approximately .904, successively nitrating said light oil at a temperature not exceeding 20° Centigrade with acid solutions consisting of nitric acid, sulphuric acid and water, rapidly increasing the temperature of the oil to approximately 70° centigrade after each nitration step and maintaining such temperature in each instance for approximately one-half hour, cooling the treated oil following each nitration step to a temperature not exceeding 30° centigrade, separating the treated oil from the spent acids after each nitration, treating the nitrated oil after each nitration step with neutralizing caustic soda solutions, and as a final step washing for approximately one-half hour the completely nitrated oil with hot water having a temperature of substantially 65° centigrade.

2. The process of manufacturing a nitro-compound which comprises distilling coal tar at temperatures ranging approximately from 95° to 115° Centigrade to produce a light oil therefrom having an average specific gravity of approximately .862, then raising the specific gravity of said oil by reflux distillation to approximately .904, then treating the oil with a fat destroying solution, then prenitrating the oil at a temperature of approximately 20° Centigrade with an acid solution consisting approximately of 70%  $H_2SO_4$ , 20%  $HNO_3$  and 10%  $H_2O$ , then raising the temperature of the prenitrated oil to approximately 70° centigrade and maintaining such temperature for approximately one-half hour, then decreasing the temperature of the prenitrated oil to substantially 30° centigrade, then separating the spent acids from the partially nitrated oil, then completing the prenitration of the latter by treating and neutralizing same with a 2% caustic soda solution and allowing the prenitrated oil to settle for approximately eight hours, then completing the nitration process at a temperature of approximately 20° centigrade with an acid solution consisting approximately of 60%  $H_2SO_4$ , 35%  $HNO_3$  and 5%  $H_2O$ , then raising the temperature of the mixture to approximately 70° centigrade and maintaining such temperature for approximately one-half hour during which period the mixture is kept in motion, then cooling the mixture to substantially 20° centigrade and allowing the same to settle for approximately four hours, then drawing off the nitrated oil from the spent acids, then treating and neutralizing the nitrated oil with a 2% to 5% solution of caustic soda until a neutral point is reached, then washing the neutralized nitrated oil with hot water having a temperature of substantially 65° centigrade for approximately one-half hour, and as a final step allowing the washed nitrated oil to settle for approximately two hours.

JAMES F. O'BRIEN. 135